# EUROPEAN PATENT SPECIFICATION

(11) **EP 0 558 178 B1**
(45) Date of publication and mention of the grant of the patent: **26.03.1997**
(21) Application number: 93300361.8
(22) Date of filing: 20.01.1993
(51) Int. Cl.: H01F 1/37

(54) **Magnetically permeable composition and soft magnetic component**
Magnetisch permeabele Zusammensetzung und weichmagnetisches Teil
Composition magnétiquement perméable et composant magnétique

(30) Priority: 28.02.1992 JP 78679/92; 10.08.1992 JP 234267/92
(43) Date of publication of application: 01.09.1993
(73) Proprietor: KUREHA KAGAKU KOGYO KABUSHIKI KAISHA, Chuo-ku Tokyo 103 (JP)
(72) Inventor: Tada, Masahito, c/o Kureha Kagaku Kogyo K.K., Tokyo 103 (JP); Suzuki, Keiichiro, c/o Kureha Kagaku Kogyo K.K., Tokyo 103 (JP)
(74) Representative: Kyle, Diana

(56) References cited:
- US-A- 4 268 430

## Description

### FIELD OF THE INVENTION AND RELATED ART

The present invention relates to a polyarylene sulfide resin composition excellent in permeability and a magnetic component shaped therefrom.

Polyarylene sulfide resin is an engineering plastic having excellent heat resistance, chemical resistance and electrical insulating property and, because of such properties, has been recently used in a wide scope of industries of, e.g., electrical, electronics and automobiles.

Of these, a permeable magnetic composition containing a powdery soft magnetic material dispersed in a binder of polyarylene sulfide resin is being considered for use as various magnetic components, such as coils, inductors and filters, by taking advantage of small mold shrinkage characteristics in addition to the heat resistance, chemical resistance and the electrical insulation properties of the polyarylene sulfide see US-A-4,268,430. As the soft magnetic material, Ni-Zn-based ferrite is particularly suitable for use in circuit components for medium frequency or high frequency ranges.

Hitherto, it has been practiced to increase the content of the soft magnetic powder in the composition in order to obtain a molded product having a high permeability. However, it has been difficult to increase the permeability of a composition comprising Ni-Zn-based ferrite as the magnetic material and polyarylene sulfide as the binder by increasing the content of the Ni-Zn-based ferrite.

### SUMMARY OF THE INVENTION

An object of the present invention is to provide a composition comprising polyarylene sulfide resin and a Ni-Zn-based ferrite having a high permeability which has not been realized by this type of composition.

Selection of a magnetic material having a higher permeability in its sintered state than the Ni-Zn-based ferrite for dispersion in a resin does not necessarily provide a resin composition having a higher permeability. As a result of our study, it has been discovered that a Ni-Zn-Cu-based ferrite of a specific composition as described below provides a composition having a high permeability when combined with polyarylene sulfide resin.

According to the present invention, there is provided a permeable magnetic composition, comprising 5 - 30 wt. parts of polyarylene sulfide resin and 70 - 95 wt. parts of Ni-Zn-Cu-based ferrite powder providing a total of 100 wt. parts together with the polyarylene sulfide resin, said Ni-Zn-Cu-based ferrite having a composition represented by the following formula (1):

NiₐZn_{b}Cu_{c}Fe₂O_{d},

wherein a, b, c and d are numbers satisfying 0.10 ≤ a ≤ 0.70, 0.10 ≤ b ≤ 0.80, 0.10 ≤ c ≤ 0.35 and 3.97 ≤ d ≤ 4.20.

These and other objects, features and advantages of the present invention will become more apparent upon a consideration of the following description of the preferred embodiments of the present invention taken in conjunction with the accompanying drawing.

### BRIEF DESCRIPTION OF THE DRAWING

Figures 1 and 2 are a perspective view and a sectional view, respectively, of a coil and a core encapsulated in Examples 5 and 6.

### DETAILED DESCRIPTION OF THE INVENTION

In Ni-Zn based ferrite, it is well known that too much or too little Ni or Zn fails to provide a high permeability. This is also true in Ni-Zn-Cu based ferrite. More specifically, it is appropriate that the parameter a representing the nickel (Ni) content is in the range of 0.10 - 0.70, preferably 0.15 - 0.50, more preferably 0.17 - 0.30. It is appropriate that the parameter b representing the zinc (Zn) content is in the range of 0.10 - 0.80, preferably 0.40 - 0.75, more preferably 0.50 - 0.70.

Similarly as the parameters a and b, too large or too small a parameter c representing the copper (Cu) content fails to provide a high permeability and the required range therefor is rather narrower than a and b. More specifically, it is appropriate that the parameter c is in the range of 0.10 - 0.35, preferably 0.15 - 0.30, more preferably 0.17 - 0.25. Below 0.10 or in excess of 0.35, it is difficult to obtain the product obtained through, e.g., injection or compression molding with an increased permeability.

Further, in the formula (1), it is appropriate that the parameter d representing the oxygen content is in the range of 3.97 - 4.20, preferably 3.98 - 4.15, more preferably 3.99 - 4.10. Below 3.97 or in excess of 4.20, the resultant product obtained through, e.g., injection or compression molding is caused to have a lower electrical insulating property, so that it becomes difficult to retain a high permeability in a high frequency region.

The Ni-Zn-Cu-based ferrite powder used in the present invention may preferably have an average particle size (diameter) according to the light scattering method (as measured by using Model "LA-500" available from Horiba Seisakusho K.K.) in the range of 3 - 200 µm, more preferably 5 - 200 µm. If the average particle size is below 3 µm, the composition is caused to have an excessively high melt viscosity, and it becomes difficult to form a molded product having a satisfactory appearance. Further, a smaller particle size tends to provide a smaller permeability. If the ferrite powder has an average particle size in excess of 200 µm, it becomes difficult to form a small size product and is liable to promote the wearing of a mold surface.

The Ni-Zn-Cu-based ferrite powder can be surface-treated with a known surface treating agent, such as a silane coupling agent, a titanate coupling agent, an aluminum coupling agent, or a phosphorus-based coupling agent.

Herein, the polyarylene sulfide resin refers to a polymer comprising at least 50 wt. %, preferably at least 70 wt. %, more preferably at least 90 wt. %, of a recurring unit represented by (̵Ar-S)̵, wherein -Ar- denotes an arylene group.

It is particularly preferred to use a polyarylene sulfide having a substantially linear structure formed from a monomer (or monomer mixture) comprising a bi-functional monomer-because of an excellent toughness. It is however possible to use a polyarylene-sulfide having a partially crosslinked structure or subjected to curing for increasing the melt viscosity as far as the mechanical properties are not impaired thereby.

A preferred example of the recurring unit (̵Ar-S)̵ is a p-phenylene sulfite unit represented by

The polyarylene sulfide may be a homopolymer, a random copolymer or a block copolymer. The copolymer may preferably comprise at least 50 wt. %, particularly at least 60 wt. %, of the p-phenylene sulfide having the structure shown above and at most 50 wt. %, particularly at most 40 wt. %, of at least one of m-phenylene sulfide unit, diphenylene sulfide unit, tri-functional phenyl sulfide unit, naphthalene sulfide unit, phenyl ketone phenyl sulfide unit, phenyl sulfone unit, phenyl ether phenyl sulfide unit, phenyl sulfone phenyl sulfide unit, and phenyl ketone phenyl ketone sulfide unit respectively represented by the following structural formulae: and

The polyarylene sulfide resin may preferably have a melt viscosity of 1 - 200 Pa.S (10 - 2000 poise), more preferably 2 - 120 Pa.S (20 - 1200 poise), further preferably 2.5 - 100 Pa.S (25 - 1000 poise), as measured at a temperature of 310 °C and a shear rate of 10³/sec.

The magnetic composition of the present invention comprises the above Ni-Zn-Cu-based ferrite in an amount of 70 - 95 wt. parts, preferably 75 - 93 wt. parts, and the polyarylene sulfide in an amount of 5 - 30 wt. parts, preferably 7 - 25 wt. parts, providing a total of 100 wt. parts together with the Ni-Zn-Cu-based ferrite. If the ferrite powder is less than 70 wt. parts, the permeability is lowered. In excess of 95 wt. parts, the composition becomes fragile.

The magnetic composition of the present invention can further contain 0 - 25 wt. % of a thermoplastic resin other than the polyarylene sulfide resin, such as polyamide resin, polyphenylene ether resin, polyether ether ketone, polyether ketone, polycarbonate or polystyrene, or a thermosetting resin, such as epoxy resin or a cured product thereof.

The magnetic composition according to the present invention can further contain an inorganic filler or fibrous reinforcing material, such as glass fiber, potassium titanate, silicon carbide, ceramic fiber, silicon nitride or asbestos, or an organic fibrous reinforcing material, such as aramide fiber.

It is particularly preferable to add epoxidized silicone oil into the composition of the present invention so as to improve the adhesiveness to a coil or a terminal electrode. By the addition, it is possible to suppress a separation from such a coil or terminal electrode or occurrence of a crack in the molded product even when subjected to a thermal impact, e.g., by re-flowing soldering. The epoxidized silicone oil may preferably be added in an amount of 0.1 - 5 wt. %, more preferably 0.2 - 2 wt. %.

So as to retain the basic properties of the permeable magnetic composition according to the present invention, it is preferred that the total amount of the Ni-Zn-Cu ferrite powder and the polyarylene sulfide resin occupies at least 85 wt. %, more preferably at least 95 wt. %, further preferably at least 97 wt. % of the composition.

The molding or shaping method applicable to the composition is not particularly limited but may preferably be one of applying a high pressure, such as injection molding or compression molding. For example, the injection molding may preferably be performed while applying a pressure of 400 - 3000 kgf/cm², more preferably 500 - 2000 kgf/cm² at a temperature which may be 15 - 100 °C higher than the melting point of the polyarylene sulfide resin.

The permeable magnetic composition according to the present invention may suitably be used for production of, e.g., magnetic components, suitable for use as or use in coil and core, inductor, rotary transformer, EMI filter, and balun requiring a high permeability and electrical insulation.

### [Examples]

Evaluation of compositions prepared in Examples and Comparative Examples was performed in the following manner.

### (Preparation of test piece)

A pellet-form composition in each Example was supplied to an injection molding machine ("PS-10E", available from Nissei Jushi K.K.) to form a toroidal core having an outer diameter of 36 mm, an inner diameter of 24 mm and a thickness of 10 mm by injection molding under the conditions of a cylinder temperature of 340 °C, a nozzle temperature of 340 °C, an injection pressure of 1500 kgf/cm² and a mold temperature of 160 °C.

### (Measurement of permeability)

A polyester-coated copper wire of 0.3 mm in diameter was wound about the toroidal core in 165 turns, and the inductance was measured at 100 KHz by using an impedance analyzer ("HP4192A", available from Yokogawa Hewlett-Packard K.K.). From the impedance, the permeability µ was calculated by the following equation:$\text{µ = (L x} {\text{l}}_{̲} {\text{}}_{\text{1}} {\text{x 10}}^{\text{7}} {\text{)/(4πn}}^{\text{2}} \text{S),}$ wherein L denotes the inductance, l₁ denotes a magnetic path length, n denotes the number of coil turns (= 165), and S denotes a core diameter. The length l₁ is calculated by the following equation:${\text{l}}_{̲} {\text{}}_{\text{1}} \text{= (} {\text{l}}_{̲} {\text{}}_{\text{d}} \text{-} {\text{l}}_{̲} {\text{}}_{\text{s}} \text{)/log(} {\text{l}}_{̲} {\text{}}_{\text{d}} \text{/} {\text{l}}_{̲} {\text{}}_{\text{s}} \text{) x π,}$ wherein l_{d} denotes the core outer diameter and lₛ denotes the core inner diameter.

### Example 1

13.5 kg of Ni-Zn-Cu-based ferrite powder (average particle size: 11 µm) having a composition represented by the chemical formula Ni_{0.19}Zn_{0.63}Cu_{0.18}Fe₂O_{4.00} and 1.5 kg of linear phenyl sulfide homopolymer (melt viscosity: about 20 Pa.s (200 poise), melting point: 290 °C) were blended in a 20 liter-Henschel mixer and melt-kneaded through a twin-screw kneading extruder to prepare a composition in the form of pellets. A toroidal core was molded from the composition and the permeability thereof was measured in the above-described manner, whereby a value of 14.8 was obtained.

The outline of the composition and the permeability of the molded product are summarized in the following Table 1 together with those of other Examples and Comparative Examples which will be described hereinafter.

**Table 1**

| | NiₐZn_{b}Cu_{c}Fe₂O_{d} | | | | | | Permeability [H/m] |
|---|---|---|---|---|---|---|---|
| | a | b | c | d | Content (%) | Dav.* (µm) | |
| Ex.1 | 0.19 | 0.63 | 0.18 | 4.00 | 90 | 11 | 14.8 |
| " 2 | 0.20 | 0.58 | 0.22 | 4.01 | 90 | 10 | 15.7 |
| " 3 | 0.63 | 0.31 | 0.15 | 4.09 | 90 | 12 | 11.7 |
| " 4 | 0.27 | 0.67 | 0.16 | 4.10 | 90 | 9 | 13.3 |
| " 6 | 0.20 | 0.58 | 0.22 | 4.01 | 85 | 10 | 10.2 |
| Comp. Ex.1 | 0.36 | 0.62 | 0 | 3.98 | 90 | 3 | 11.0 |
| " 2 | 0.60 | 0.37 | 0 | 3.97 | 90 | 10 | 10.8 |
| " 3 | 0.30 | 0.30 | 0.41 | 4.01 | 90 | 11 | 10.5 |

| | | | | | | | |
|---|---|---|---|---|---|---|---|
| * Dav. = average particle size | | | | | | | |

### Example 2

A composition was prepared from 13.5 kg of Ni-Zn-Cu-based ferrite powder represented by the formula Ni_{0.20}Zn_{0.58}Cu_{0.22}Fe₂O_{4.01} and 1.5 kg of the linear phenylene sulfide homopolymer and formed into a toroidal core in the same manner as in Example 1. The core provided a permeability shown in Table 1.

### Example 3

A composition was prepared from 13.5 kg of Ni-Zn-Cu-based ferrite powder represented by the formula Ni_{0.63}Zn_{0.31}Cu_{0.15}Fe₂O_{4.09} and 1.5 kg of the linear phenylene sulfide homopolymer and formed into a toroidal core in the same manner as in Example 1. The core provided a permeability shown in Table 1.

### Example 4

A composition was prepared from 13.5 kg of Ni-Zn-Cu-based ferrite powder represented by the formula Ni_{0.27}Zn_{0.67}Cu_{0.16}Fe₂O_{4.10} and 1.5 kg of the linear phenylene sulfide homopolymer and formed into a toroidal core in the same manner as in Example 1. The core provided a permeability shown in Table 1.

### Example 5

A chip-form ferrite core for an inductor having a shape as shown in Figure 1 (perspective view) and Figure 2 (sectional view) was provided. The core had two end disks 1 each having a diameter of 3 mm and a thickness of 1 mm and a through hole 2 to pass a lead wire therethrough. The disks 1 were connected with a cylindrical bar 3 having a length of 3 mm and a diameter of 1.8 mm. A copper wire was wound in the form of a coil 4 about the bar 3 and the two ends thereof were passed through the disks 1 to form leads 4a and 4b.

The coil and core were placed in a mold as an insert and encapsulated except for the leads 4a and 4b with the composition of the above Example 1 to form a molded product in the form of a rectangular parallelepiped measuring 7 mm x 4 mm x 4 mm by using an injection molding machine ("JT-40", available from Nippon Seiko-sho K.K.). The molded product was immersed for 10 seconds in a solder bath at 260 °C and then taken out for inspection of the appearance. As a result, no crack was observed at the parts contacting the leads of the molded product, and no surface abnormality was observed either. Further, no change in inductance was observed before and after the immersion in the solder bath.

### Example 6

12.75 kg of Ni-Zn-Cu-based ferrite represented by the chemical formula Ni_{0.20}Zn_{0.58}Cu_{0.22}Fe₂O_{4.01} and 2.25 kg of the polyphenylene sulfide resin were blended in a 20 liter-Henschel mixer, and 112.5 g of epoxidized silicone oil was added and mixed therewith. The resultant mixture was melt-kneaded through a twin-screw kneading extruder to prepare a composition in the form of pellets, which was then molded into a toroidal core in the above-described manner. The core provided a permeability shown in Table 1 above.

A coil and a core identical to those used in Example 5 were encapsulated with the composition of this Example in a similar manner as in Example 5 to form a similar molded product. The molded product was immersed for 10 seconds in a solder bath at 260 °C and then taken out for inspection of the appearance. As a result, no crack was observed at the parts contacting the leads of the molded product, and no surface abnormality was observed either. Further, no change in inductance was observed before and after the immersion in the solder bath.

### Comparative Example 1

A composition was prepared from 13.5 kg of Ni-Zn-based ferrite powder represented by the formula Ni_{0.36}Zn_{0.62}Fe₂O_{3.98} and 1.5 kg of the linear phenylene sulfide homopolymer and formed into a toroidal core in the same manner as in Example 1. The core provided a permeability shown in Table 1.

### Comparative Example 2

A composition was prepared from 13.5 kg of Ni-Zn-based ferrite powder represented by the formula Ni_{0.60}Zn_{0.37}Fe₂O_{3.97} and 1.5 kg of the linear phenylene sulfide homopolymer and formed into a toroidal core in the same manner as in Example 1. The core provided a permeability shown in Table 1.

### Comparative Example 3

A composition was prepared from 13.5 kg of Ni-Zn-Cu-based ferrite powder represented by the formula Ni_{0.30}Zn_{0.3}Cu_{0.41}Fe₂O_{4.01} and 1.5 kg of the linear phenylene sulfide homopolymer and formed into a toroidal core in the same manner as in Example 1. The core provided a permeability shown in Table 1.

As described above, according to the present invention, there is provided a polyarylene sulfide resin composition showing a high permeability.

From the composition, it is possible to obtain magnetic components suitable for use as or use in coil-core, inductor, rotary transformer, EMI filter and balun. These components or articles can be suitably used when they are required to show excellent heat-resistance and chemical resistance.

## Claims

1. A permeable magnetic composition, comprising 5 - 30 wt. parts of polyarylene sulfide resin and 70 - 95 wt. parts of Ni-Zn-Cu-based ferrite powder providing a total of 100 wt. parts together with the polyarylene sulfide resin, said Ni-Zn-Cu-based ferrite having a composition represented by the following formula (1):
NiₐZn_{b}Cu_{c}Fe₂O_{d},
wherein a, b, c and d are numbers satisfying 0.10 ≤ a ≤ 0.70, 0.10 ≤ b ≤ 0.80, 0.10 ≤ c ≤ 0.35 and 3.97 ≤ d ≤ 4.20.

2. A composition according to Claim 1, wherein the numbers a - d satisfy 0.15 ≤ a ≤ 0.50, 0.40 ≤ b ≤ 0.75, 0.15 ≤ c ≤ 0.30, and 3.98 ≤ d ≤ 4.15.

3. A composition according to Claim 1 or 2, comprising 7 - 25 wt. parts of the polyarylene sulfide resin and 75 - 93 wt. parts of the Ni-Zn-Cu-ferrite powder.

4. A composition according to any one of Claims 1 - 3, further containing 0.1 - 5 wt. % of epoxidized silicone oil.

5. A magnetic component, comprising a molded product of a permeable magnetic composition according to any preceding claim.

## Patentansprüche

1. Eine magnetische Zusammensetzung mit Permeabilität, umfassend 5 - 30 Gewichtsteile eines Polyarylensulfidharzes und 70 - 95 Gewichtsteile eines Ferritpulvers auf der Grundlage von Ni-Zn-Cu, wobei dieser Anteil zusammen mit dem Anteil an Polyarylensulfidharz 100 Gewichtsteile ausmacht und der besagte Ferrit auf der Grundlage von Ni-Zn-Cu eine Zusammensetzung aufweist, welche der nachstehenden Formel (1) entspricht:
NiₐZn_{b}Cu_{c}Fe₂O_{d},
in welcher a,b,c und d Zahlenwerte darstellen, welche die nachstehenden Beziehungen befriedigen: 0.10 ≤ a ≤0.70, 0.10 ≤ b ≤ 0.80, 0.10 ≤ c ≤ 0.35 und 3.97 ≤ d ≤ 4.20.

2. Eine Zusammensetzung gemäß Anspruch 1, in welcher die Zahlenwerte für a bis d die nachstehenden Beziehungen befriedigen: 0.15 ≤ a ≤ 0.50, 0.40 ≤ b ≤ 0.75, 0.15 ≤ c ≤ 0.30 und 3.98 ≤ d ≤ 4.15.

3. Eine Zusammensetzung gemäß Anspruch 1 oder 2, umfassend 7 - 25 Gewichtsteile des Polyarylensulfidharzes und 75 - 93 Gewichtsteile des Ni-Zn-Cu-Ferrits.

4. Eine Zusammensetzung gemäß irgendeinem der Ansprüche 1 bis 3, welche außerdem 0.1 - 5 Gew% epoxidiertes Silikonöl enthält.

5. Eine magnetische Komponente, welche ein geformtes Produkt aus einer magnetischen Zusammensetzung mit Permeabilität nach irgendeinem der vorstehenden Ansprüche umfaßt.

## Revendications

1. Composition magnétique perméable comprenant 5-30 parties en poids d'une résine de sulfure de polyarylène et 70-95 parties en poids d'une poudre de ferrite à base de Ni-Zn-Cu, fournissant un total de 100 parties en poids conjointement avec la résine de sulfure de polyarylène, ladite ferrite à base de Ni-Zn-Cu possédant une composition représentée par la formule suivante (1) :
NiₐZn_{b}Cu_{c}Fe₂O_{d},
a, b, c et d étant des nombres satisfaisant à 0,10 ≤ a ≤ 0,70, 0,10 ≤ b ≤ 0,80, 0,10 ≤ c ≤ 0,35 et 3,97 ≤ d ≤ 4,20.

2. Composition selon la revendication 1, dans laquelle les nombres a-d satisfont à 0,15 ≤ a ≤ 0,50, 0,40 ≤ b ≤ 0,75, 0,15 ≤ c ≤ 0,30, et 3,98 ≤ d ≤ 4,15.

3. Composition selon la revendication 1 ou 2, comprenant 7-25 parties en poids de résine de sulfure de polyarylène et 75-93 parties en poids de poudre de ferrite de Ni-Zn-Cu.

4. Composition selon l'une quelconque des revendications 1-3, contenant en outre 0,1-5 % en poids d'huile silicone époxydée.

5. Composant magnétique constitué par un produit moulé formé d'une composition magnétique perméable selon l'une quelconque des revendications précédentes.
